

3,043,736

**METHOD FOR MAKING ADDITIVE FILTERS**  
George P. Touey, Kingsport, Tenn., assignor to Eastman Kodak Company, Rochester, N.Y., a corporation of New Jersey  
No Drawing. Filed Mar. 2, 1959, Ser. No. 796,259  
11 Claims. (Cl. 156—152)

This invention relates to methods for making tobacco smoke filtering material and elements thereof suitable for use in cigarettes, pipes, cigarette holders and cigar holders. More particularly, the invention is concerned with improvements in making filters of the kind disclosed in my application Serial No. 432,931, now U.S. Patent No. 2,881,770, of which the instant invention is a continuation-in-part.

In my patent just referred to, I have shown filters of substantially increased efficiency without equivalent increase in pressure drop by providing a filter which contains certain finely divided solids in the smoke channels provided by the spacing of adjacent filaments. I further have shown in my patent that when carbon powder, particularly activated carbon powder is employed as the finely divided deposit on the filaments, unusual efficiency is obtained.

In my new filters, as just referred to, it is desirable that the additive be applied in a rapid efficient manner. Also, the finely divided carbon is preferably sufficiently adhered to the filaments so that it will not dust off, come loose in the smoker's mouth or otherwise present such type difficulty. Accordingly, it is believed apparent that providing improved methods for making carbon containing filters of the type just referred to represents a highly desirable result. After extended investigation I have found certain improved methods for manufacturing such filters.

This invention, therefore, has as one object an improved method for the production of cigarette smoke filters consisting of a bundle of substantially longitudinally oriented textile filaments infused with finely divided carbon particles. Another object is to provide methods of the class indicated for increasing the bonding of the particles onto the filament filter. A still further object is to make an additive filter which is capable of removing nicotine, tars and other deleterious components of cigarette smoke without causing the smoke to be dry or distasteful. Another object is to provide improved methods which are efficient and effective, yet relatively economical and simple in operation. Other objects will be apparent from the present specification and claims.

As referred to above and as disclosed in my patent concerning, in general, the filter product, my filter product comprises a longitudinally oriented mass of substantially lengthwise aligned filaments, the spacing of substantially all groups of adjacent filaments providing minute passages for smoke therethrough, said mass carrying finely divided carbon particles, said particles occupying positions in and partially blocking said passages whereby a substantial portion of the smoke is impinged either on the filaments, or on the carbon.

I have found there are certain methods which advantageously may be employed in manufacturing my filter product. In the broader aspects of the present invention, methods as follows may be used:

Thus, for example, the carbon powder can be blown onto the filaments or it can be applied as a slurry in aqueous media or in a volatile organic vehicle or a plasticizer for the filaments. Another procedure is to apply the carbon powder to the filaments by means of a latex emulsion. Still another way of applying the carbon is to wet the surface of the filaments with an adhesive or a plasticizer before exposing them to a powder spraying

device. Preferably, the carbon is continuously applied to an opened and banded moving tow. That is to say, tow from a supply roll is opened to debundle the filaments and provide a larger and more uniform tow cross section, and the opened tow is spread uniformly to a much larger width of e.g., 8 times its original width, thereby exposing substantially all of the filaments to material, i.e. plasticizer, issuing from a dispenser adjacent which the tow passes. The carbon may be added before, simultaneously with, or after the plasticizer, preferably with or after.

Certain of the preferred methods are further illustrated in greater detail in the following examples:

15

*Example I*

A continuous filament tow of yarn-type cellulose acetate of 5 denier per filament with a total denier of 100, 20 000, and 9 crimps per inch was used. The tow was pulled from a package of tow over stationary tensioning fingers and into a tensioning device functioning to provide tow opening as the first phase of filament separation. The device employed was of the type employing a pair of driven rolls to place under tension tow positioned in the ratch between the driven rolls and a pair of retarded rolls upstream of the driven rolls. The device was equipped with the improved reciprocating striker as disclosed and claimed in Smith pending U.S. patent application Serial 25 No. 416,010, filed March 15, 1954, now Patent No. 2,790,208. Upon being released from the nip of the positively driven tension rolls into a zone of relative relaxation, i.e. relatively little tension, the tow bloomed through inherent forces manifested upon the return of 30 the tow to its original position.

The partially opened tow of several thousand cellulose acetate filaments was slowly pulled over a compressed air banding device as disclosed in application Serial No. 356, 983, filed May 25, 1953, by Wallace T. Jackson, now 40 Patent No. 2,737,688. The banding device momentarily spread out the fibers to a width of six inches. While the tow was in this spread condition it was sprayed with a highly agitated slurry of one part activated bone charcoal powder in five parts dimethoxyethylphthalate plasticizer.

45 After this spreading and spraying treatment the tow was uniformly collected and fed to a garniture for forming the filaments carrying carbon particles into a filter. The tow was fed into the garniture through a shaping horn which served to condense the conditioned tow back 50 into the shape of a cord or cylinder. The machine then wrapped the formed filaments with paper and cut it into rods similar in size to a standard size cigarette. The rods contained 1 part carbon powder, 5 parts plasticizer and 20 parts cellulose acetate by weight. After the filter 55 rods were given a short heat treatment to cause partial solvation of the acetate fibers by the plasticizer they were readily cut into 15 mm. filter tip lengths. These tips were attached by means of an adhesive tape to a standard brand of king-size cigarette available on the retail market

60 in the U.S. and shortened by 15 mm. to compensate for the length of the filter. The cigarettes were smoked on a smoking machine similar in design and operation to the smoking machine described by J. A. Bradford, W. R. Harlan and M. R. Hanmer in Industrial and Engineering Chemistry, vol. 28, pp. 836-9 (1936). The collected smoke was analyzed for nicotine and tars. The results of the smoking experiment were compared with those obtained from smoking the same brand of cigarettes containing 65 15 mm. filter tips made from the same tow of cellulose acetate fibers plasticized with dimethoxyethylphthalate without the addition of carbon.

70

| Type of cigarette filter tip (15 mm.)                                | Mg. of tars <sup>1</sup> | Mg. of nicotine <sup>1</sup> |
|----------------------------------------------------------------------|--------------------------|------------------------------|
| Plasticized cellulose acetate tow                                    | 130                      | 20                           |
| Plasticized cellulose acetate tow containing 4% bone charcoal powder | 108                      | 17                           |

<sup>1</sup> Obtained from the collected smoke of ten filtered cigarettes. NOTE. Moisture of the tobacco in each of the cigarettes equals 12.2%.

The cigarettes containing the acetate tow filters had an average pressure drop of 3.9 inches; the cigarettes containing the filters of cellulose acetate tow and bone charcoal powder had an average pressure drop of 4.1 inches, where pressure drop is measured as inches of water pressure developed when air is pulled through the cigarette at the rate of 17.5 ml. per second. This method of pressure drop has been described by G. P. Touey in *Ind. and Eng. Chemistry*, vol. 27, page 1789 (1955).

#### Example II

A loose, i.e., partially opened crimped continuous filament tow of cellulose acetate yarn containing approximately 10,000 fibers of 8 denier per filament was pulled through a bath containing a highly agitated slurry of commercially available activated wood charcoal in water. When dried, the tow contained 10% of charcoal powder by weight uniformly dispersed throughout. The carbon impregnated tow was processed into filter rods in a garniture as described in Example I and the resulting rods were cut into 15 mm. lengths. The filter tips so produced were attached to standard brand king-size cigarettes shortened by 15 mm. cigarettes and ten of these filter tipped cigarettes were smoked on the smoking machine. The collected smoke was analyzed for nicotine and tars. A control, consisting of the same brand of cigarettes tipped with filters made from the 8 denier per filament tow containing no carbon was also smoked on the smoking machine and the collected smoke was analyzed in the same manner for nicotine and tars.

|                                                 | Mg. of tars | Mg. of nicotine |
|-------------------------------------------------|-------------|-----------------|
| Acetate tow filter                              | 132         | 21              |
| Acetate tow filter containing 10% wood charcoal | 122         | 17              |

NOTE. Moisture of the tobacco in each of the cigarettes equals 12.3%.

The cigarettes containing the acetate tow filters had an average pressure drop of 3.7 inches; the cigarettes containing the filters of cellulose acetate tow and wood charcoal powder had an average pressure drop of 3.9 inches, where pressure drop is measured as explained in Example I above.

#### Example III

A tow of cellulose acetate yarn containing approximately 40,000 fibers of 3 denier per filament was spread out to a width of six inches and sprayed with a 10% solution of a waterbase adhesive. While the tow was still spread out and wet with the adhesive it was sprayed with a commercially available finely divided lampblack powder and then rolled back into its original form. The impregnated tow was processed into filter rods and the rods were cut into 15 mm. lengths. The filter tips, containing 9% carbon based on the weight of the acetate fibers, were attached to standard brand king-size cigarettes shortened by 15 mm. to compensate for the length of the filter. Ten of these cigarettes were smoked on the smoking machine. The collected smoke was analyzed for nicotine and tars. A control consisting of the same brand of cigarettes tipped with a filter of the 3 denier per filament tow containing the adhesive but no lampblack carbon powder was also smoked on the smoking machine and the collected smoke was analyzed in the same manner for nicotine and tars.

|                                                   | Mg. of tars | Mg. of nicotine |
|---------------------------------------------------|-------------|-----------------|
| Acetate tow filter                                | 125         | 18              |
| Acetate tow filter containing 9% lampblack powder | 113         | 15              |

NOTE.—Moisture of the tobacco in each of the cigarettes equals 12.0%.

- The cigarette containing the acetate tow filters had an average pressure drop of 4.0 inches; the cigarettes containing the filters of cellulose acetate tow and lampblack powder had an average pressure drop of 4.2 inches, where pressure drop is measured as explained in Example I above.
- 10 For water base bonding media I may employ a water solution of dextrin, polyvinyl alcohol, starch, a water-soluble cellulose derivative, water-soluble natural gums, sugars, melamine formaldehyde and urea formaldehyde resins.
- 15 However, in most instances I prefer to employ an organic plasticizer capable of partially dissolving the cellulose acetate filaments such as described in Example I. Illustrations of other suitable plasticizers are: glycerol di- and triacetate, glycerol di- and tripelargonate, propylene 25 glycol mono- and diacetate, di(methoxyethyl)phthalate, triethyl citrate, acetyl-triethyl citrate and methylphthalyl-ethyl glycolate.

#### Example IV

- 30 A tow of cellulose acetate yarn containing approximately 6,000 fibers of five denier per filament was pulled over a compressed air device which spread out the fibers to a width of six inches. While the tow was in this spread condition it was sprayed with a mixture consisting of 1 part polyvinyl acetate emulsion (55% solids-45% water), 1 part powdered activated charcoal, and 2 parts water. The tow was then fed through a cigarette make-up machine which cut and paper wrapped it into rods of 8.1 mm. diameter and 71 mm. lengths. They were "cured" 35 by heating to 100° C. for 30 minutes. The dried rods contained 39% activated charcoal and 21.4% polyvinylacetate. They were then cut into 13-mm. tips, and attached to an American king-size cigarette which had been shortened by 13 mm. Ten filtered cigarettes were smoked on a smoking machine similar in design and operation to the smoking machine described by J. A. Bradford, W. R. Harlan and H. R. Hammer in *Industrial and Engineering Chemistry*, vol. 28, pp. 836-9 (1936). The gaseous phase of the smoke was collected and analyzed for total aldehyde. Ten unfiltered cigarettes were smoked, and the 45 gaseous phase analyzed in the same manner for use as a control. The filtered smoke contained 25% less aldehydes than the unfiltered smoke.

#### Example V

- 50 A tow of cellulose acetate yarn containing approximately 6,000 fibers of five denier per filament, was sprayed with a mixture consisting of 1 part polyvinyl isobutyrate emulsion (50% solids), 1 part powdered activated charcoal, and 2 parts water. The tow was processed into filter tips, attached to cigarettes, and analyzed as in Example IV. The dried tips contained 11.7% polyvinyl isobutyrate and 23.4% activated charcoal. They removed 19% of the aldehydes from the gaseous phase of cigarette smoke.

#### Example VI

- 65 A tow of cellulose acetate yarn containing approximately 12,000 fibers of five denier per filament was sprayed with a mixture consisting of 1 part polyvinyl acetate emulsion (55% solids-45% water), 1 part activated charcoal and 2 parts water. The tow was processed into filter tips, attached to cigarettes and analyzed as in Example IV. The dried tips contained 13.4% of polyvinyl acetate and 24.4% activated charcoal. They removed 20% of the aldehydes from the gaseous phase 70 of cigarette smoke.

## 5

## Example VII

A tow of cellulose acetate yarn containing approximately 12,000 fibers of five denier per filament was sprayed with a mixture consisting of 1 part polyvinyl acetate emulsion (55% solids-45% water) and 2 parts water. The tow was processed into filter tips, attached to cigarettes and analyzed as in Example IV. The tips contained 22.4% polyvinyl acetate. They removed less than 4% of the aldehydes from cigarette smoke. The pressure drop of these filtered cigarettes was approximately the same as the pressure drop of the filtered cigarettes described in the earlier examples and only slightly higher than that of the unfiltered control cigarettes.

Another type of method of applying activated carbon involves the use of molten materials such as stearyl alcohol and the like shown in companion copending application Touey et al., Serial No. 701,310. That is, a mixture of a material such as activated carbon with melted stearyl alcohol, for example, when sprayed on the fibers, produces a much more efficient filter than can be made by prior art methods. The presence of the carbon apparently increases the atomization efficiency of the spray head so that finer, sharper particles of the melted material and carbon are produced, and the tendency toward agglomeration is very appreciably reduced. While I prefer to use an activated carbon in combination with melted stearyl alcohol, stearic acid, fatty glycerides, polyoxyethylene or paraffin waxes, it is also possible to use other solid additives of small particle size to produce this increase in atomization efficiency with respect to the melt material. Examples of these other solid powders may be found in silica gel, rice starch, calcium carbonate, and aluminum oxide and aluminum hydroxy stearate. For a more complete understanding of this feature, reference is made to the following examples:

## Example VIII

A mixture is made by adding 20 grams of activated carbon (Darco G-60) to 80 grams of molten stearyl alcohol. This mixture is sprayed on a plasticized cigarette tow prepared from crimped 5 denier per filament 55,500 total denier acetate. An add-on of 15% by weight of mix based on tow weight was made. When tested on a Phipps and Byrd smoking machine using the total smoke solids procedure, a removal of 50% of the smoke particles was accomplished.

## Example IX

A cellulose acetate tow of 5 denier per filament, 55,500 total denier was sprayed with a mixture of stearyl alcohol and finely powdered activated carbon to give an add-on, based on tow weight, of 22.5% stearyl alcohol and 4.5% carbon. Removals as determined in Example VIII averaged 53% for a 15 mm. tip having a pressure drop of 2.7 inches of water.

## Example X

A mixture of stearyl alcohol and activated carbon was sprayed on a 2.1 denier per filament, 44,400 total denier acetate tow to give an add-on of 12.5% stearyl alcohol and 2.5% carbon. Removals as determined by Example VIII averaged 48% for a standard 15 mm. tip having a pressure drop of 2.6 inches of water.

## Example XI

An acetate tow of 2.1 denier per filament, 44,000 total denier was sprayed with a mixture of stearic acid and activated charcoal to give an add-on of 12.5% stearic acid and 2.5% carbon. When tested in the usual manner, a standard 15 mm. tip gave an average removal of 52% at a 2.7-inch pressure drop.

In carrying out the operation of these methods the type of carbon employed is not a critical factor. Rather, the form of the carbon is more important. The carbon should be in a powdered form so that it can be readily slurried in a liquid or passed through a spraying nozzle.

## 6

Any source of carbon which passes this requirement can, therefore, be employed. Such commercial carbon powders as bone charcoal, coconut charcoal, wood charcoal or lampblack carbon may be employed. Also, as apparent from the above examples, various types of emulsions of carbon or graphite may be employed.

In the case wherein the carbon powder is dusted on the spread out tow after it has been sprayed with plasticizer, one might wish to increase the tackiness of the plasticizer. This can readily be done by dissolving 3 to 20% of certain low molecular weight polymers in the plasticizer before it is sprayed on the tow. This would create a more tacky surface on the tow which in turn would form a better bond between the carbon particles and the fiber surfaces. Low molecular weight organic solvent soluble polymers such as polyvinyl acetate, polyvinyl pyrrolidone, and the esters of polyacrylic acid are ideally suited for this purpose. Also, a low viscosity type of organic solvent soluble cellulose ester could be used as a thickener and tackifier for the plasticizer. All of these compounds are readily soluble in the plasticizers already mentioned for cellulose acetate tow filters. They are particularly effective with glycerol di- and triacetate.

As apparent from the above examples, unusually good results have been obtained with filters prepared from a crimped continuous filament tow of cellulose acetate fibers sprayed with certain plasticizers in accordance with the preferred embodiments of this invention. However, in the broader aspects of the invention in certain instances the usefulness of the methods extends to other synthetic fibrous filters, including those prepared from fibers of viscose, polyamides and polyesters, where the fibers are continuous and in substantial longitudinal alignment and are coextensive with the body of the filter.

Some of the methods described above will give filters which will remove a substantial amount of low molecular weight aldehydes from cigarette smoke. It is generally believed that aldehydes such as acetaldehyde and acrolein have a harmful and irritating effect upon the membranes of the throat and mouth; hence it is desirable that their concentration in cigarette smoke be reduced.

In my preferred embodiment and method I apply the additive to continuous crimped cellulose acetate filaments of a total denier within the range of 40,000 to 120,000 and of denier per filament of below 16 and preferably below 5. I have found that the present methods work very well on filaments of a denier of 2-3. The filaments would be crimped, for example at least 8 crimps per inch and preferably 12 or more crimps. The amount, percentage by weight of additive, based on total weight of additive plus weight of filament applied by my methods would usually be at least 10% and may be as high as 40% in many instances.

The invention has been described in detail with particular reference to preferred embodiments thereof, but it will be understood that variations and modifications can be effected within the spirit and scope of the invention as described hereinabove and as defined in the appended claims.

I claim:

1. The method for the continuous manufacture of tobacco smoke filters which comprises continuously withdrawing crimped continuous tow of synthetic spun filaments from a package of such tow, banding the tow to a width of at least six inches, applying to the banded tow both bonding agent and powdered additive, reforming the tow thus treated into the desired filter shape and wrapping the filter with a wrapper.

2. A method in accordance with claim 1 wherein the tow consists essentially of cellulose acetate filaments of a denier per filament of less than 8 and of a total denier of less than 120,000.

3. A method in accordance with claim 1 wherein the bonding agent is a plasticizer from the group consisting of glycerol di- and triacetate, glycerol di- and tripropionate, propylene glycol mono- and diacetate, di(meth-

oxyethyl)phthalate, triethyl citrate, acetyl-triethyl citrate and methylphthalylethyl glycolate and the additive is finely divided carbon.

4. A method in accordance with claim 1 wherein the bonding agent is a latex material essentially comprised of a polyvinyl polymeric compound.

5. The method for the manufacture of filters from spun filaments which comprises substantially continuously withdrawing crimped continuous spun cellulose acetate filaments from a package thereof, banding such filaments to a width of at least 8 inches, applying to the banded filaments a molten mixture of a high molecular weight compound from the group consisting of esters, acids and alcohols which are normally solid at room temperature but which are normally fluid at above 50° C. and which molten high molecular weight compound has incorporated therein a content of finely divided solid additive, reforming the banded filaments thus treated into the desired filter shape and wrapping the periphery of the filter with a wrapper.

6. The method in accordance with claim 5 wherein the additive is finely divided carbon.

7. The method in accordance with claim 5 wherein the compound is stearyl alcohol and the finely divided additive is carbon.

8. The method for manufacturing tobacco smoke filters which comprises withdrawing crimped continuous cellulose acetate filaments of a denier per filament of less than 5 and a total denier of less than 100,000 from a package of such filaments, banding such filaments to a width of at least six inches, applying to the banded filaments both a bonding media and activated carbon particles, the bonding media being such that it will not materially deactivate

the activated carbon additive, reforming the filaments thus treated into the desired filter shape and applying a wrapper around the circumference of the filter.

9. In a method of making tobacco smoke filters from crimped continuous cellulose acetate filaments wherein the filaments are banded into an opened up condition, the step which comprises spraying the opened up filaments with an emulsion essentially comprised of a polyvinyl compound from the group consisting of polyvinyl acetate and polyvinyl isobutyrate which polyvinyl compound has mixed therewith powdered charcoal and water.

10 15 15. In a method of making tobacco smoke filters from crimped continuous cellulose acetate filaments wherein the filaments are banded into an opened up condition, the step which comprises spraying the opened up filaments with a mixture of plasticizer and finely divided carbon.

16 20 11. A method for adding activated carbon to a cellulose acetate tow wherein the tow is first sprayed with an organic plasticizer containing 3 to 20% of a dissolved polymeric material and then it is dusted with a fine powder of the activated carbon.

#### References Cited in the file of this patent

#### UNITED STATES PATENTS

|           |                 |                |
|-----------|-----------------|----------------|
| 2,373,296 | Donnelly        | Apr. 10, 1945  |
| 2,763,267 | Muller          | Sept. 18, 1956 |
| 2,768,913 | Hiler           | Oct. 30, 1956  |
| 2,774,680 | Hackney et al.  | Dec. 18, 1956  |
| 2,794,239 | Crawford et al. | June 4, 1957   |
| 2,794,480 | Crawford et al. | June 4, 1957   |
| 2,815,761 | Shearer         | Dec. 10, 1957  |